



US008650756B2

(12) **United States Patent**  
**Wadley et al.**

(10) **Patent No.:** **US 8,650,756 B2**  
(45) **Date of Patent:** **Feb. 18, 2014**

(54) **MANUFACTURE OF LATTICE TRUSS  
STRUCTURES FROM MONOLITHIC  
MATERIALS**

(75) Inventors: **Haydn N. G. Wadley**, Keswick, VA (US); **John J. Wetzel**, Charlottesville, VA (US); **Yellapu V. Murty**, Charlottesville, VA (US)

(73) Assignee: **University of Virginia Patent Foundation**, Charlottesville, VA (US)

(\*) Notice: Subject to any disclaimer, the term of this patent is extended or adjusted under 35 U.S.C. 154(b) by 0 days.

(21) Appl. No.: **12/479,408**

(22) Filed: **Jun. 5, 2009**

(65) **Prior Publication Data**

US 2009/0286100 A1 Nov. 19, 2009

**Related U.S. Application Data**

(63) Continuation-in-part of application No. 12/447,166, filed as application No. PCT/US2007/022733 on Oct. 26, 2007, now Pat. No. 8,176,635.

(60) Provisional application No. 61/088,584, filed on Aug. 13, 2008, provisional application No. 60/855,089, filed on Oct. 27, 2006, provisional application No. 60/963,790, filed on Aug. 7, 2007.

(51) **Int. Cl.**  
**B21D 47/00** (2006.01)

(52) **U.S. Cl.**  
USPC ..... **29/897.31**; 29/897; 29/897.3; 29/897.32; 29/897.312; 29/897.35; 52/633; 52/634; 52/636

(58) **Field of Classification Search**  
USPC ..... 52/633-638, 693, 696, 643, 655.1, 646, 52/745.2, 651.11, 645; 29/897, 897.3,

29/897.31, 897.312, 897.35, 525.01, 557, 29/558, 840.046, 840.05, 846.6  
See application file for complete search history.

(56) **References Cited**

**U.S. PATENT DOCUMENTS**

|                 |   |         |                      |          |
|-----------------|---|---------|----------------------|----------|
| 5,690,035 A     | * | 11/1997 | Hatayama et al. .... | 105/452  |
| 6,226,944 B1    | * | 5/2001  | Peshkam et al. ....  | 52/309.8 |
| 6,537,682 B2    | * | 3/2003  | Colligan .....       | 428/593  |
| 6,938,383 B2    | * | 9/2005  | Morris et al. ....   | 52/95    |
| 2006/0283129 A1 | * | 12/2006 | Salhaney .....       | 52/633   |

\* cited by examiner

*Primary Examiner* — Brian Glessner

*Assistant Examiner* — Patrick Maestri

(74) *Attorney, Agent, or Firm* — Vincent M DeLuca; Robert J. Decker

(57) **ABSTRACT**

Methods and systems to manufacture bonded corrugation truss-based structures. This allows the ability to change the dimensions of the individual structural features of the corrugations, i.e. thickness of the core, face sheet thickness, relative density of the core, and the alloys. The nodal design which provides ideal stress/strain distribution for in-plane and out-of-plane loading. The node has a curved/smooth triple point intersection which in turn can provide best load transfer interface with high integrity/toughness. The bonded corrugation truss based structure can be continuous to any length only limited by the volume of the extrusion billet and the press capacity. An aspect of the bonded corrugation structures may include friction stir welding of the face sheets or any fusion welding of panels with edge members for strengthening allows fabrication of panels of any width and length. Bonding panels enables the fabrication of structures of any width.

**18 Claims, 26 Drawing Sheets**



**FIG. 1A****FIG. 1B****FIG. 1C**

**FIG. 2A****FIG. 2B**



FIG. 3



FIG. 4A

**FIG. 4B****FIG. 5**



FIG. 6B

**FIG. 7****FIG. 8A****FIG. 8B** $\epsilon = 0\%$ **FIG. 8C** $\epsilon = 5\%$  $\epsilon = 10\%$  $\epsilon = 10\%$  $\epsilon = 15\%$  $\epsilon = 15\%$  $\epsilon = 20\%$  $\epsilon = 20\%$  $\epsilon = 25\%$  $\epsilon = 25\%$ **FIG. 8F****FIG. 8G**

**FIG. 9A****FIG. 9B****FIG. 9C****FIG. 9D****FIG. 10A****FIG. 10B**

**FIG. 11**

(a) impulse loading (stage I)



FIG. 12A



**FIG. 12B**



**FIG. 12C**

**FIG. 13A****FIG. 13B**

**FIG. 13C****FIG. 13D**



FIG. 14A



FIG. 14B



FIG. 14C



FIG. 15A



FIG. 15B





FIG. 17A



FIG. 17B



FIG. 18A



FIG. 18B





FIG. 19A

| Standoff Distance | Extruded Corrugated Panel Back Face Deflection | Equivalent Mass Plate (17 mm Thick) Back Face Deflection |
|-------------------|------------------------------------------------|----------------------------------------------------------|
| 15 cm             | 55 mm (Failure)                                | 47 mm                                                    |
| 19 cm             | 32 mm                                          | 36 mm                                                    |
| 22 cm             | 25 mm                                          | 30 mm                                                    |
| 25 cm             | 21.5 mm                                        | 25.5 mm                                                  |

FIG. 19B



FIG. 20A



FIG. 20B



FIG. 21A



FIG. 21B



FIG. 22A



FIG. 22B



FIG. 23A



FIG. 23B



FIG. 24A



FIG. 24B

### Failure Modes of Corrugated Panels

| Standoff | Defining Failure Mode                                                         |
|----------|-------------------------------------------------------------------------------|
| 25 cm    | Crack Along Clamped Edge of Panel Parallel to Corrugations                    |
| 22 cm    | Crack Along Weld Edge of Panel Parallel to Corrugations                       |
| 19 cm    | Crack Development on Back Facesheet Weld Edge Parallel to Corrugations        |
| 15 cm    | Catastrophic Failure in Center and Clamped Edge Perpendicular to Corrugations |

FIG. 25

# MANUFACTURE OF LATTICE TRUSS STRUCTURES FROM MONOLITHIC MATERIALS

## RELATED APPLICATIONS

This application claims priority under 35 USC §119(e) to U.S. Provisional Application Ser. No. 60/088,584, filed Aug. 13, 2008, entitled "Use of a Multifunctional Aluminum Alloy Sandwich Panel for Mine Blast Protection," and this application also claims priority under 35 USC §120 as a continuation-in-part application of U.S. application Ser. No. 12/447,166, filed Apr. 24, 2009, which is a national stage filing of International Application No. PCT/US2007/022733, filed Oct. 26, 2007, which claims priority from U.S. Provisional Application Ser. No. 60/855,089 filed Oct. 27, 2006, entitled "Manufacture of Lattice Truss Sandwich Structures from Monolithic Materials" and U.S. Provisional Application Ser. No. 60/963,790 filed Aug. 7, 2007, entitled "Manufacture of Lattice Truss Sandwich Structures from Monolithic Materials;" all of the disclosures of which are hereby incorporated by reference herein in their entirety.

## GOVERNMENT SUPPORT

Work described herein was supported by Federal Grant No. ONR Grant Nos. N00014-01-1-1051 and N00014-07-1-0764, awarded by Office of Naval Research. The Government has certain rights in the invention.

## BACKGROUND OF THE INVENTION

Lightweight sandwich panel structures consisting of low density cores and solid facesheets are widely used in engineering applications. Cellular core structures based upon honeycomb topologies are often used because of their high compressive strength-to-weight ratios and high bending stiffness. These honeycomb structures are close-celled with limited access into the core regions. The cores may be attached to the facesheets or plates by conventional joining methods, such as adhesive bonding, brazing, diffusion bonding and welding. Recently, lattice truss structures have been explored as an alternate cellular core topology. Pyramidal lattice truss structures are usually fabricated from high ductility alloys by folding a perforated metal sheet along the perforations, creating accordion-like structures. Conventional joining methods such as brazing or laser welding are then used to bond the core to solid facesheets, forming sandwich structures. The lattice topology, core relative density, and parent alloy mechanical properties, along with the bond strengths, determine the mode of truss deformation and, therefore, the out-of-plane and in-plane mechanical properties of these structures.

The design of the core-facesheet node interface is of the utmost importance. Ultimately, this dictates the maximum load that can be transferred from the facesheets to the core. Node bond failure has been identified as a failure mode for sandwich structures, especially metallic honeycombs. However, analogous node failure modes have been observed in sandwich panels utilizing tetragonal and pyramidal lattice truss cores during shear loading. Assuming sufficient core-faceplate bond (facesheet-bond) strength and ductility, when sandwich panels are subjected to intense shear or bending loads, the nodes transfer forces from the facesheets to the core members and the topology for a given core relative density dictates the load carrying capacity. When the node-facesheet interfacial strength is compromised by poor joint design or

inadequate bonding methods, node bond failure occurs resulting in premature failure of the sandwich panel. Numerous factors determine the robustness of nodes, including joint composition, microstructure, degree of porosity, geometric effects (which control stress concentrations) and the nodes' contact area.

Micromechanical models for the stiffness and strength of pyramidal lattice truss cores, comprising elastic-plastic struts with perfect nodes have been recently developed. These models assumed that the trusses are connected to rigid face sheets and are of sufficiently low aspect ratio that bending effects make a negligible contribution to the stiffness and strength. These micromechanical models also assume the node strength is the same as the parent metal alloy. However, the measured elastic moduli rarely reach the predicted values because of variations in the length of the trusses and small initial departures from straightness introduced by manufacturing processes.

The design of the core-to-facesheet interface in honeycomb sandwich panels is of utmost importance. Ultimately, this dictates the amount of load that can be transferred from the face sheets to the core. This is even more critical for lattice-based cores since they can have a smaller node area than honeycombs of the same core density. Node bond failure has been identified as a key catastrophic failure mode for metallic honeycomb sandwich structures (See Bitzer, 1997). Similar node robustness problems have been observed in lattice-based sandwich structures. When sandwich panels are subjected to shear or bending loads, the nodes transfer forces from the facesheets to the core, assuming adequate node bond strength exists, and the topology for a given core relative density dictates the load carrying capacity. When the core-facesheet interface strength is compromised by poor joint design or weak bonding methods, node failure occurs and catastrophic failure of the sandwich panel results. Although numerous factors (including joint composition, microstructure, degree of porosity, and geometric constraints) determine the robustness of nodes, the node contact area serves as a critical limiting factor in determining the maximum force that can be transmitted across the core-facesheet interface.

Initial efforts to fabricate millimeter scale structures employed investment casting of high fluidity casting alloys such as copper/beryllium (See Wang et al., 2003), aluminum/silicon (See Deshpande et al., 2001, Deshpande and Fleck, 2001, Wallach and Gibson, 2001, Zhou et al., 2004), and silicon brass (See Deshpande and Fleck, 2001). Investment casting begins with the creation of a wax or polymer pattern of the lattice truss sandwich structure. The sandwich structure is attached to a system of liquid metal gates, runners, and risers that are made from a casting wax. The whole assembly is coated with ceramic casting slurry. The pattern is then removed and the empty (negative) pattern filled with liquid metal. After solidification, the ceramic, gates, and runners are removed, leaving behind a lattice based sandwich structure of homogeneous metal. However, the tortuosity of the lattices made it difficult to fabricate high-quality investment-cast structures at the low relative density (2-10%) needed to optimize sandwich panel constructions (See Chiras et al., 2002). In addition, the inherent low quality of as-cast metals resulted in sandwich structures that lacked the robustness required for the most demanding structural applications (See Sugimura, 2004).

The toughness of many wrought engineering alloys is evidenced by development of alternative fabrication approaches based upon perforated metal sheet folding (See Sypeck and Wadley, 2002). These folded truss structures could be bonded to each other or to facesheets by either transient liquid phase

(TLP) bonding or micro welding techniques to form lattice-truss sandwich panels. Panels fabricated with tetrahedral (See Sypeck and Wadley, 2002, Rathbun et al., 2004, Lim and Kang, 2006) and pyramidal lattice-truss (See Zok et al., 2004, Quechillalt and Wadley, 2005, McShane et al., 2006, Radford, et al. 2006) topologies have been made by the folding and brazing/TLP bonding method. However, the node bond strength and the topology for a given core relative density may dictate the load-carrying capacity. While these structures are much more robust than their investment cast counterparts, their robustness may be dictated by the quality of the bond between the core and facesheets.

A detailed description of the fabrication approach for making 6061 aluminum alloy lattice truss structures can be found in Multifunctional Periodic Cellular Solids and the Method of Making the Same (PCT/US02/17942, filed Jun. 6, 2002), Method for Manufacture of Periodic Cellular Structure and Resulting Periodic Cellular Structure (PCT/US03/16844, filed May 29, 2003), and Methods for Manufacture of Multilayered Multifunctional Truss Structures and Related Structures therefrom (PCT/US2004/004608, filed Feb. 17, 2004), of which all of the PCT Applications are hereby incorporated by reference herein in their entirety. Briefly, these patents describe a folding process used to bend perforated sheets to create a single or multiple-layered lattice truss structures. The folding is accomplished using a paired punch and die tool or a finger break to fold node rows into the desired truss structure. The lattice truss core is then joined to facesheets via one of the previously mentioned methods to form the lattice truss sandwich structure (i.e. adhesives, welding, brazing, soldering, transient liquid phase sintering, etc.).

#### SUMMARY OF INVENTION

Provided herein are exemplary methods and systems to manufacture lattice-based sandwich structures from monolithic material. Such methods and systems eliminate the bonding process which is conventionally used to join lattice based truss cores to facesheets to form sandwich structures. This bonded interface is a key mode of failure for sandwich structures which are subjected to shear or bending loads because the nodes transfer forces from the face sheets to the core members while the topology for a given core relative density dictates the load carrying capacity (assuming adequate node-bond strength exists).

An aspect of an embodiment of the present invention comprises a core and related structures that provide very low density, good crush resistance and high in-plane shear resistance. An aspect of the truss structures may include sandwich panel cores and lattice truss topology that may be designed to efficiently support panel bending loads while maintaining an open topology that facilitates multifunctional applications.

Some aspects of various embodiments of the present invention method and system utilize, but are not limited to, novel methodologies to construct sandwich structures without using adhesives, diffusion bonding, brazing, soldering, or resistance/electron/laser welding or coupling to join the cores to the facesheets to form sandwich structures. Facesheet-core interface bond failure (e.g., facesheet-core interface) may be a key failure mode for lattice based sandwich structures. When lattice based sandwich panels are subjected to shear or bending loads, the nodes transfer forces from the face sheets to the core members (assuming adequate node bond strength exists) and the topology (for a given core relative density) dictates the load carrying capacity. However, when the node-facesheet interface strength is compromised, node failure occurs and catastrophic failure of the sandwich panel results.

Some aspects of various embodiments of the present invention method and system may utilize, but are not limited thereto, a two-step manufacturing process. A prismatic structure is extruded forming a 3D structure with a constant cross section along the path of extrusion; thereafter a secondary operation is used to selectively remove material, from the core region, forming a 3D lattice truss sandwich structure. This process can be used for any metal, including (but not limited thereto) steel, aluminum, copper, magnesium, nickel, 10 titanium alloys, etc., and is highly suited for alloys that possess limited ambient temperature ductility.

It should be appreciated that the method of manufacture/fabrication may be altered or adjusted in interest of creating a resultant structure that is ultimately desired or required.

An aspect of an embodiment of the present invention provides a method of creating a monolithic lattice truss or truss-based structure (or related structure as desired or required). The method comprising: providing a monolithic sample; extruding the monolithic sample to selectively remove material along a first path; and machining the monolithic sample to selectively remove material along a second path, wherein the first path and the second path are offset at a desired offset angle to create one or a plurality of truss unit portions. Multiple paths and various types of paths and respective locations 20 and angles may be applied as desired or required to achieve the desired method or structure.

An aspect of an embodiment of the present invention provides a method of creating a monolithic lattice truss structure (or related structure as desired or required). The method comprising: providing a monolithic sample; machining the monolithic sample to selectively remove material along a first path; and machining the monolithic sample to selectively remove material along a second path, wherein the first path and the second path are offset at a desired offset angle to create one or 30 a plurality of truss unit portions. Multiple paths and various types of paths and respective locations and angles may be applied as desired or required to achieve the desired method or structure.

An aspect of an embodiment of the present invention provides a monolithic lattice truss structure (or related structure as desired or required). The structure comprising: one or a plurality of truss unit portions, wherein the truss unit portions have the same metallurgical and microstructural properties.

An aspect of an embodiment of the present invention provides a structure that is manufactured or fabricated in whole or in part and by any one or combination of the manufacturing or fabrication methods discussed herein.

Provided herein are exemplary methods and systems to manufacture bonded corrugation truss based structures from monolithic material. Relatively narrow panels with several cells can manufactured from monolithic materials, but are limited because of the narrow width which is imposed by the limits of current extrusion technology. The Truss-based sandwich structures can be welded using friction stir welding to 50 avoid melting the material and weakening the welds. If other welding methods are used it is desirable to include the use of a vertical side member in the structure to reinforce the welded region. The vertical side members may be thickened.

An aspect of an embodiment of the present invention comprises a core and related structures that provide very low density, good crush resistance and high in-plane shear resistance. An aspect of the truss structures may include sandwich panel cores and that may be designed to efficiently support panel bending loads while maintaining an open topology that 55 facilitates multifunctional applications.

Some aspects of various embodiments of the present invention method and system may utilize, but are not limited

thereto, a two-step manufacturing process. Corrugation truss based structures are created by extruding monolithic structures; thereafter the extrusions can be joined using adhesives, diffusion bonding, brazing, soldering, or resistance/electron/laser/friction stir welding or coupling or welded together to form a panel of any width. This process can be used for any metal, including (but not limited thereto) steel, aluminum, copper, magnesium, nickel, titanium alloys, etc., and is highly suited for alloys that possess limited ambient temperature ductility.

It should be appreciated that the method of manufacture/fabrication may be altered or adjusted in interest of creating a resultant structure that is ultimately desired or required.

An aspect of an embodiment of the present invention provides a method of creating a monolithic truss-based structure (or related structure as desired or required). The method comprising: providing monolithic samples; extruding the monolithic samples to selectively remove material along the extruded path; and welding the extrusions together by the process of friction stir welding.

An aspect of an embodiment of the present invention provides a method of creating a monolithic truss structure (or related structure as desired or required). The method comprising: providing a monolithic samples; extruding the monolithic samples to selectively remove material along the extruded path; including a vertical side member in the extruded structures; and joining the extruded structures using adhesives, diffusion bonding, brazing, soldering, or resistance/electron/laser/friction stir welding or coupling or welded together to form a panel of any width such that vertical side members are located at the interfaces of the joined extruded structures.

An aspect of an embodiment of the present invention provides a method of creating a monolithic truss structure (or related structure as desired or required). The method comprising: providing a monolithic samples; extruding the monolithic samples to selectively remove material along the extruded path such that the extrusion nodes have a curved or smoothed triple point interface with the facesheet; including a vertical side member in the extruded structures; and joining the extruded structures using adhesives, diffusion bonding, brazing, soldering, or resistance/electron/laser/friction stir welding or coupling or welded together to form a panel of any width; such that vertical side members are located at the interfaces of the joined extruded structures.

An aspect of an embodiment of the present invention provides a method of creating a monolithic lattice truss structure (or related structure as desired or required). The method comprising: providing a monolithic samples; extruding the monolithic samples to selectively remove material along the extruded path such that the extrusion nodes have a curved or smoothed triple point interface with the facesheet; including a vertical side member in the extruded structures; and joining the extruded structures using adhesives, diffusion bonding, brazing, soldering, or resistance/electron/laser/friction stir welding or coupling or welded together to form a panel of any width such that vertical side members are located at the interfaces of the joined extruded structures; repeating the process to manufacture several such panels; and the panels are stacked upon each other and bonded by various metallurgical or adhesive methods to create a multilayered structure.

An aspect of an embodiment of the present invention provides a method of creating a monolithic lattice truss structure (or related structure as desired or required). The method comprising: providing a monolithic samples; extruding the monolithic samples to selectively remove material along the extruded path such that the extrusion nodes have a curved or

smoothed triple point interface with the facesheet; including a vertical side member in the extruded structures; and joining the extruded structures using adhesives, diffusion bonding, brazing, soldering, or resistance/electron/laser/friction stir welding or coupling or welded together to form a panel of any width such that vertical side members are located at the interfaces of the joined extruded structures; repeating the process to manufacture several such panels; and the panels either in single or multilayer form are edge supported (e.g., clamped).

10 An aspect of an embodiment provides a method of creating bonded corrugation truss based structures. The method comprising: providing a monolithic sample; extruding the monolithic sample to selectively remove material, which yields a first corrugation panel; extruding another the monolithic sample to selectively remove material, which yields a second corrugation panel; and laterally coupling the first and second corrugation panels in communication with one another to form a single continuous plurality panel.

An aspect of an embodiment comprises a panel, the panel 20 comprising: a first monolithic corrugated panel and a second monolithic corrugated panel that are laterally coupled in communication with one another to form a single continuous plurality panel.

25 These and other objects, along with advantages and features of the invention disclosed herein, will be made more apparent from the description, drawings and claims that follow.

#### BRIEF DESCRIPTION OF THE DRAWINGS

30 The accompanying drawings, which are incorporated into and form a part of the instant specification, illustrate several aspects and embodiments of the present invention and, together with the description herein, and serve to explain the 35 principles of the invention. The drawings are provided only for the purpose of illustrating select embodiments of the invention and are not to be construed as limiting the invention.

FIGS. 1(A)-(C) provide schematic illustrations of three 40 stages of the manufacturing method utilizing two arrays of channels EDM cut into a monolithic block of metal forming a pyramidal lattice truss sandwich structure.

FIGS. 2(A)-(B) provide schematic illustrations of two of the stages of the manufacturing method utilizing a single 45 array of channels EDM cut into an extruded prismatic sandwich structure forming a pyramidal lattice truss sandwich structure.

FIG. 3 provides a photographic depiction of a pyramidal lattice sandwich structure which was EDM cut from a 6061 aluminum alloy extrusion.

FIGS. 4(A)-(B) provide schematic illustrations of two of the stages of the manufacturing method of a double-layer pyramidal lattice sandwich structure with aligned nodes between adjacent layers and a double array of channels EDM 55 cut into an extruded double-layer prismatic sandwich structure.

FIG. 5 provides a schematic illustration of the extrusion process used to produce 6061 aluminum corrugated sandwich structures.

FIGS. 6(A)-(B) provide schematic illustrations of the 60 regions in the corrugated core that are removed by electro discharge machining to create a pyramidal lattice core sandwich panel structure.

FIG. 7 provides a photographic depiction of an extruded/electro discharge machined pyramidal lattice sandwich structure with a core relative density of 6.2%.

FIG. 8(A) graphically illustrates the compressive stress versus strain response. Predictions of the stress for inelastic

buckling and plastic yielding of the trusses are also shown. FIGS. 8(B)-(G) provide photographic depictions of the lattice deformation at strain levels ( $\epsilon$ ) of 0, 5, 10, 15, 20 and 25%, respectively.

FIG. 9(A) graphically illustrates the shear stress versus shear strain response. Predictions of the stress for inelastic buckling and plastic yielding of the trusses are also shown. FIGS. 9(B)-(D) provide photographic depictions of the lattice deformation at strain levels ( $\gamma$ ) of 0, 6 and 12%, respectively.

FIGS. 10(A)-(B) graphically illustrates the normalized (a) compression and (b) shear stiffness measurements, respectively, versus strain.

FIG. 11 provides a schematic illustration of one embodiment of a sandwich structure of the p-JBD system interacting with a jet.

FIGS. 12(A)-(C) provide schematic illustrations of an embodiment of a sandwich structure demonstrating blast or explosion mitigation in response to an explosion. FIGS. 12(A)-(C) provide the impulse loading stage, core crushing stage, and panel bending stage, respectively.

FIGS. 13(A)-(D) provide schematic illustrations of an embodiment of a sandwich structure 1201 demonstrating projectile arresting capabilities in response to a projectile, which provides various rupture and fracture details.

FIGS. 14(A)-(C) provides a schematic illustration the typical extrusion process used to cut a monolithic block of metal forming a pyramidal lattice truss sandwich structure, a cross section of a pyramidal lattice truss sandwich structure, and three nodes with a curved or smooth triple point interface with the facesheet.

FIGS. 15(A)-(B) provide a schematic illustration of the friction stir welding technique used to join extruded prismatic sandwich structures to form a panel and a cross section of the panel.

FIG. 16(A)-(B) provides a photographic depiction extrusion of extruded and friction stir welded corrugated core 6061-T6 aluminum sandwich panel, and a close-up of the panel cross section highlighting the weld line and the dimensions of the core, the facesheets, and the vertical side member.

FIG. 17(A) graphs hardness of the corrugation plurality panels in MPa as a function of distance from the weld.

FIG. 17(B) graphs the true stress in MPa as a function of true strain for both the parental material.

FIGS. 18(A)-(B) provide a schematic illustration and a photograph depiction of the "Black Widow" blast testing rig used to evaluate the mine blast resistance of the corrugation panels.

FIGS. 18(C)-18(H) provide a schematic illustration depicting the process for constructing the "wet sand" charge, which is used for simulating mine blasts.

FIGS. 19(A)-(B) provide a graph and a chart of the back facesheet deflection of the corrugation panel and a mass equivalent solid panel at different standoff distances using the "Black Widow" blast testing rig.

FIG. 20(A)-(B) provides photographs of corrugation plurality panels (FIG. 7(A)) and mass equivalent solid panels (FIG. 20(B)) subjected to the black widow blast testing rig at different standoff distances.

FIGS. 21(A)-(B) provide photographs of a corrugation plurality subjected to the black widow blast testing rig at a 25 cm standoff. Additionally, FIG. 21(A) provides an enlarged partial view highlighting tearing along the region where the corrugation plurality panel is clamped to the rig. FIG. 21(B) shows partial close-up images of the cross section of the corrugation plurality panel.

FIGS. 22(A)-(B) provide photographs of a corrugation plurality subjected to the black widow blast testing rig at a 22

cm standoff. Additionally, FIG. 22(A) provides an enlarged partial view highlighting tearing along the region where the corrugation plurality panel is clamped to the rig. FIG. 22(B) shows partial close-up images of the cross section of the corrugation plurality panel.

FIGS. 23(A)-(B) provide photographs of a corrugation plurality subjected to the black widow blast testing rig at a 19 cm standoff. Additionally, FIG. 23(A) provides an enlarged partial view highlighting tearing along the region where the corrugation plurality panel is clamped to the rig. FIG. 23(B) shows partial close-up images of the cross section of the corrugation plurality panel.

FIGS. 24(A)-(B) provide photographs of a corrugation plurality subjected to the black widow blast testing rig at a 15 cm standoff. Additionally, FIG. 24(A) highlights tearing along the region where the corrugation plurality panel is clamped to the rig. FIG. 24(B) shows partial close-up images of the cross section of the corrugation plurality panel.

FIG. 25 provides a summary table of the results of the corrugation plurality panels subjected to the black widow blast testing rig.

## DETAILED DESCRIPTION OF THE INVENTION

As described earlier, a variety of lattice topologies can be fabricated from ductile metals using current fabrication methods that rely on cutting, stamping and/or bending processes to form the desired lattice core, which is then subsequently bonded to facesheet by a variety of methods including, but not limited to, adhesives, diffusion bonding, brazing, soldering or resistance/electron/laser welding, coupling, etc. The design of the core-to-facesheet interface is of utmost importance. Ultimately, this dictates the amount of load that can be transferred from the facesheets to the core, and, ultimately, supported by the truss assembly.

Provided herein, an aspect of an embodiment provides methods and systems that result in sandwich structures with highly robust nodes that can be manufactured from any metal, including, but not limited to steel, aluminum, copper, magnesium, nickel, titanium alloy, etc. These methods are well-suited for alloys that possess limited ambient temperature formability.

The following are exemplary methods and systems of various embodiments of the present invention that can be used to fabricate lattice truss sandwich structures (or any structure as desired/required) from any metal, thus greatly expanding the realm of metals that can be fabricated into cellular structures, as the aforementioned methods (adhesives, diffusion bonding, brazing, soldering or resistance/electron/laser welding, etc.) could only have been fabricated from alloys. In addition, since there is no metallurgical or microstructural discontinuity at the truss-facesheet (truss-faceplate) interface region, the likelihood of corrosion is greatly reduced.

In an exemplary and non-limiting embodiment of an aspect of the present invention, a pyramidal lattice sandwich structure is formed from a solid monolithic sample 1, such as a piece of metal, but not limited thereto. The initial monolithic sample 1 can be sheet, plate, ingot, billet, powder compact, or slurry, or the like, form depending on the size of the final sandwich structure or any desired/required structure. The following is a description for the manufacture of a pyramidal lattice. It should also be appreciated, however, that tetrahedral, Kagome, cone, frustum, or other lattice-based truss structures may be manufactured via this method as desired or required. FIG. 1(A) shows an example of a solid, monolithic sample 1. FIG. 1(B) shows an example of a triangulated pattern machined in the y-direction. This pattern can be

machined via electro discharge machining, drilling including laser drilling and other ablative removal techniques in which material is melted or evaporated, cut, water jet cutting, chemical dissolution methods or any other suitable operation. At this point, the structure has the form of a 2D prismatic sandwich structure 2 with facesheets 11 and a consistent cross-section along the y-axis. FIG. 1(C) shows an example of a triangulated pattern machined in the x-direction. Again, this pattern can be machined via electro discharge machining, cutting or any other suitable operation. The result of the combination of these two processes is a 3D lattice truss sandwich structure 3 with facesheets 11 enclosing truss units 12, forming nodes 13 where a truss units 12 interfaces with a facesheet 11. The truss units 12 comprise of a plurality of legs or ligaments 14. The legs may have a variety of shapes such as straight or curved and may have a variety of cross-sections. The plurality of truss units 12 form an array of truss units. While the y-direction path and the x-direction path are shown as substantially straight, it should be appreciated that the paths may be curved or shaped as desired or required. For instance, the array of truss units and panels (or any related components of the resultant structure) may be fabricated so that the truss units and panels (or any related components) may be contoured or shaped as desired or required. Moreover, while the various paths (x, y, and z) as illustrated appear to be substantially orthogonal or perpendicular respectively with one another, it should be appreciated that any respective angles may be implemented as desired or required for the desired or required fabrication process or resultant truss and/or panel structure. In an embodiment, the monolithic sample 1 may comprise at least one select material as desired or required. In an embodiment, the select material may comprise, for example but not limited thereto, ceramic, polymer, metal, metal alloy, and/or any combination of composites thereof (or any material(s) as desired or required. It should be appreciated that the monolithic sample may be machined along a plurality of paths, such as two or more as desired or required. It should be appreciated that the monolithic sample may be extruded along a plurality of paths, such as two or more as desired or required. The area that the faceplate or facesheet and truss units intersect form an interface region. In an embodiment, the interface region has the same metallurgical and microstructural properties. In an embodiment, the truss units have nodes wherein the nodes have the same metallurgical and microstructural properties as the truss unit. In an embodiment, the extruding or machining or both the extruding and machining create the truss units of varying relative density.

In an exemplary and non-limiting embodiment of an aspect of the present invention, a pyramidal lattice sandwich structure is formed from an extruded prismatic structure. The extruded prismatic structure can take on a variety of shapes, dependent only upon the desired topology of the final sandwich structure or any desired/required structure. Again, the following is a description for the manufacture of a pyramidal lattice. It is envisioned, however, that tetrahedral, Kagome, cone, frustum, or other lattice-based truss structures may be manufactured via this method. FIG. 2(A) shows an example of an extruded triangulated pattern 21 (extruded direction is the y-direction), with facesheets 11. FIG. 2(B) shows an example of a triangulated pattern machined in the x-direction of the extruded topology, the combination of these two steps producing a pyramidal lattice sandwich structure. Again, this pattern can be machined via electro discharge machining, cutting, drilling including laser drilling and other ablative removal techniques in which material is melted or evaporated, water jet cutting, chemical dissolution methods or any other suitable operation.

other suitable operation resulting in the 3D lattice truss sandwich structure 22 with facesheets 11 enclosing truss units 12, forming nodes 13 where truss legs or ligaments 14 interface with a facesheet 11. The truss units 12 comprise of a plurality of legs or ligaments 14. The legs may have a variety of shapes such as straight or curved and may have a variety of cross-sections. The plurality of truss units 12 form an array of truss units. While the y-direction path and the x-direction path are shown as substantially straight, it should be appreciate that the paths may be curved or shaped as desired or required. For instance, the array of truss units and panels (or any related components of the resultant structure) may be fabricated so that the truss units and panels (or any related components) may be contoured or shaped as desired or required. Moreover, while the various paths (x, y, and z) as illustrated appear to be substantially orthogonal or perpendicular respectively with one another, it should be appreciated that any respective angles may be implemented as desired or required for the desired or required fabrication process or resultant truss and/or panel structure. In an embodiment, the monolithic sample 1 may comprise at least one select material as desired or required. In an embodiment, the select material may comprise, for example, but not limited thereto, ceramic, polymer, metal, metal alloy, and/or any combination of composites thereof (or any material(s) as desired or required. It should be appreciated that the monolithic sample may be machined along a plurality of paths, such as two or more as desired or required. It should be appreciated that the monolithic sample may be extruded along a plurality of paths, such as two or more as desired or required. The area that the facesheet or faceplate and truss units intersect form an interface region. In an embodiment, the interface region has the same metallurgical and microstructural properties. In an embodiment, the truss units have nodes wherein the nodes have the same metallurgical and microstructural properties as the truss unit. In an embodiment, the extruding or machining or both the extruding and machining create the truss units of varying relative density.

FIG. 3 provides a photographic depiction of a pyramidal lattice sandwich structure 23 which was EDM cut from a 6061 aluminum alloy extrusion with facesheets 11 enclosing truss units 12, forming nodes 13 where truss legs or ligaments 14 interfaces with a facesheet 11.

In an exemplary and non-limiting embodiment of an aspect of the present invention, these manufacturing techniques may be used to form multi-layered sandwich panels. Again, the following is a description for the manufacture of a double-layer pyramidal lattice, however, it is envisioned that tetrahedral, Kagome, cone, frustum, or other lattice-based truss structures of any number of layers may be manufactured via this method. FIG. 4(A) shows an example of a double-layer extruded triangular pattern 31 sandwich structure (extruded direction is the y-direction). FIG. 4(B) shows an example of a triangulated pattern machined in the x-direction of the extruded topology, forming a pyramidal lattice sandwich structure. Again, this pattern can be machined via electro discharge machining, drilling including laser drilling, cutting, removing and other ablative removal techniques in which material is melted or evaporated, water jet cutting, chemical dissolution methods or any other suitable operation. The combination of these two steps produces a multi-layered 3D lattice truss sandwich structure 32, with facesheets 11 enclosing truss units 12, forming nodes 13 where truss legs or ligaments 14 interface with a facesheet 11. It is noted that the alignment of nodes 32 between adjacent layers is not a prerequisite. As with this embodiment or any embodiments discussed herein, each individual layer may be aligned or offset

## 11

any amount from adjacent layers, yielding the desired properties for the structure as a whole and the layers individually. Similarly, the truss units may have any number of legs or ligaments according to the fabrication approach. The truss units 12 comprise of a plurality of legs or ligaments 14. The legs may have a variety of shapes such as straight or curved and may have a variety of cross-sections. The plurality of truss units 12 form an array of truss units. While the y-direction path and the x-direction path are shown as substantially straight, it should be appreciated that the paths may be curved or shaped as desired or required. Moreover, while the various paths (x, y, and z) as illustrated appear to be substantially orthogonal or perpendicular respectively with one another, it should be appreciated that any respective angles may be implemented as desired or required for the desired or required fabrication process or resultant truss and/or panel structure. For instance, the array of truss units and panels (or any related components of the resultant structure) may be fabricated so that the truss units and panels (or any related components) may be contoured or shaped as desired or required. In an embodiment, the monolithic sample 1 may comprise at least one select material as desire or required. In an embodiment, the select material may comprise, for example but not limited thereto, ceramic, polymer, metal, metal alloy, and/or any combination of composites thereof (or any material(s) as desired or required. It should be appreciated that the monolithic sample may be machined along a plurality of paths, such as two or more as desired or required. It should be appreciated that the monolithic sample may be extruded along a plurality of paths, such as two or more as desired or required. The area that the faceplate/facesheet and truss units intersect form an interface region. In an embodiment, the interface region has the same metallurgical and microstructural properties. In an embodiment, the truss units have nodes wherein the nodes have the same metallurgical and microstructural properties as the truss unit. In an embodiment, the extruding or machining or both the extruding and machining create the truss units of varying relative density.

Aspects of various embodiments of the present invention provide, but are not limited to, a novel method and system to manufacture lattice-based truss sandwich structures or any desired/required structures that provides enhanced truss-facesheet interface strength by avoiding poor joint design or bonding procedures, which can cause the catastrophic failure of sandwich panels. Although numerous factors determine the robustness of joined nodes (joint composition, microstructure, degree of porosity, geometric constraints, etc.) this new method results in sandwich structures with highly robust nodes that have the equivalent metallurgical, for instance strength, ductility, chemical composition, microstructural characteristics, etc. of the parent material. Aspects of the present invention methods can be used for, but are not limited to, any solid, metal, or metal alloy, including, but not limited to steels, aluminum, copper, magnesium, nickel, titanium alloy, etc. and is highly suited for alloys which possess limited ambient temperature ductility.

This approach can be extended to other material classes. For example, various approaches have been developed for producing polymeric structures with prismatic cores that can then be fabricated via the means described heretofore, including 3D lattice truss sandwich structures. Ceramic materials with prismatic cores can also be fabricated using “green state” extrusion forming and sintering, in which the material can be laterally machined prior to or after a sintering operation. Edge-defined film fed growth also provides a means for fabricating prismatic structures of the type envisioned here from

## 12

many types of materials, including ceramics (sapphire for example) and semiconductors (such as silicon).

FIG. 11 is a schematic illustration of one embodiment of p-JBD system 100 interacting with jet 120. When jet 120 emits a jet blast (not pictured), it interacts with p-JBD 110 or the like. The thermal component of the jet blast is absorbed in to the structure of p-JBD 110 or the like and spread across its surface, and the kinetic component of the jet blast is deflected up and over p-JBD 110. As the kinetic component passes over the top of p-JBD 110 it must travel over the deployable ejector plate 140, which creates a low pressure or vacuum region (not pictured) above p-JBD 110 as the kinetic component interacts with the ambient air there. This process pulls cool air 150, brought into p-JBD 110 through inlet 130 at its base up through the p-JBD structure, thus removing the thermal component of the jet blast stored there. As a result hot air 160 is expelled out the top of p-JBD 110. It should be appreciated that in some embodiments, p-JBD 110 may be coated with a spray-on non-skid protective surface 170 or any other form of coating designed to provide traction. Passive in this context implies a system that does not necessarily require an active cooling system. Although, it should be appreciated that an active cooling system may be added, supplemented or implemented with the disclosed cooling system and related method disclosed throughout this document regarding the present invention methods and systems. As shown, the p-JBD 110 comprises a plurality of first plates 112 in communication or joined (e.g., side-by-side or laterally) with one another along with their respective second plates 111 on the back side with a core 114 disposed there between.

Further, during assembly of any of the components related with the JBD system a variety of welding or joining techniques may be applied, including, but not limited thereto, friction stir welding for effective joining. Some of the joints, particularly “lap joints” provide open paths to bare aluminum (or desired or required material) of the plates or cores (for example), which in turn may produce undesirable corrosion product in certain instances. To prevent this, optionally special sealants may be employed which are applied during welding (e.g., friction stir welding or as desired or required) to those lap joints.

FIGS. 12(A)-(C) are schematic illustration of an embodiment of a sandwich structure 1201 demonstrating blast or explosion mitigation in response to an explosion. FIGS. 45 12(A)-(C) provide the impulse loading stage, core crushing stage, and panel bending stage, respectively.

FIGS. 13(A)-(D) are schematic illustration of an embodiment of a sandwich structure 1301 demonstrating projectile arresting capabilities in response to a projectile, which provides various rupture and fracture details. As shown inserts 1305 (e.g., prism shaped) are disposed therein and filler material 1303 (e.g., elastomers) in the interstitial space of the sandwich structure 1301.

The following are exemplary methods and systems of various embodiments of the present invention that can be used to bonded corrugation truss based structures (or any structure as desired/required) from any metal, thus greatly expanding the realm of metals that can be fabricated into truss based structures, as the aforementioned methods (adhesives, diffusion bonding, brazing, soldering or resistance/electron/laser welding, etc.) could only have been fabricated from alloys. In addition, since there is no metallurgical or microstructural discontinuity at the truss-facesheet (truss-faceplate) interface region, the likelihood of corrosion is greatly reduced.

In an exemplary and non-limiting approach of an embodiment, a monolithic sample may be extruded, to form a first corrugation panel. A second monolithic sample may be

## 13

extruded to form a second corrugation panel. It should be appreciated that the monolithic samples can be aluminum, ceramic, polymer, metal, alloy, and/or any combination of composites thereof, or the like, form depending on the size of the final corrugation truss based structures or any desired/required structure. The two corrugation panels can then be laterally coupled in communication with one another to form a single continuous plurality panel. The term laterally may encompass, for example, side-by-side arrangement or at least substantially side-by-side. The corrugation panels can be coupled using adhesives, diffusion bonding, brazing, soldering or resistance/electron/laser welding, friction stir welding, coupling, etc. The above steps can be repeated to form a continuous plurality panel containing any number of corrugation panels. As discussed herein, various embodiments comprise the structure and related method for the manufacture of a corrugation plurality panel with a prismatic core shape. It should also be appreciated, however, that tetrahedral, Kagome, cone, frustum, or other truss structures may be manufactured via this method as desired or required.

FIG. 14(A) shows an example of an extrusion process whereby a monolithic sample has been extruded to form a corrugation panel 153, with a prismatic core shape 1507 (as shown in FIG. 14(B)). It should be appreciated that prior to or after any extrusions the pattern, sample, billet, panel or structure may be fabricated or manipulated by being machined via electro discharge machining, drilling including laser drilling and other ablative removal techniques in which material is melted or evaporated, cut, water jet cutting, chemical dissolution methods or any other suitable operation. At this point, as shown in FIG. 14(B), the truss based structure 1503 has the form of a single corrugation panel, with a prismatic core shape 1507, facesheets 1504 enclosing truss units 1505, forming nodes 1506 where truss units 5 interfaces with the facesheets 1504.

FIG. 14(B) shows a schematic of a 6061 aluminum alloy that has been extruded with a regular prismatic structure using a 17.8 cm diameter, 300 ton direct extrusion press at 482° C. After this extrusion step, the resulting corrugated core sandwich panel structures, i.e., truss based structure 1503, had a web thickness of 0.125 in, a core height of 0.75 in, 0.216 in thick facesheets and a web inclination angle of 60 degrees as shown in FIG. 14(B). The truss units 1505 comprise of a plurality of legs or ligaments 1511. The legs may have a variety of shapes such as straight or curved and may have a variety of cross-sections. The plurality of truss units 1505 form an array of truss units. While the y-direction path is shown as substantially straight, it should be appreciate that the path may be curved or shaped as desired or required. For instance, the array of truss units and panels (or any related components of the resultant structure) may be fabricated so that the truss units and panels (or any related components) may be contoured or shaped as desired or required. Moreover, while the various extruded paths (x, y, and z) as illustrated appear to be substantially orthogonal or perpendicular respectively with one another, it should be appreciated that any respective angles may be implemented as desired or required for the desired or required fabrication process or resultant truss and/or panel structure. In an embodiment, the monolithic sample may comprise at least one select material as desired or required. In an embodiment, the select material may comprise, for example but not limited thereto, aluminum, ceramic, polymer, metal, metal alloy, and/or any combination of composites thereof (or any material(s) as desired or required. The area that the faceplate or facesheet and truss units intersect form an interface region. In an embodiment, the interface region has the same metallurgical and micro-

## 14

structural properties. In an embodiment, the truss units have nodes wherein the nodes have the same metallurgical and microstructural properties as the truss unit. In an embodiment, the extruding or machining or both the extruding and machining create the truss units of varying relative density. In an embodiment, the nodes have curved or smooth triple point interfaces with the facesheets.

FIG. 14(C) depicts a schematic illustration of a truss unit portion 1505 with nodes 1506 that have curved or smooth triple point interfaces with the face sheet 1504.

Referring to FIG. 15, in an exemplary and non-limiting embodiment of an aspect of the present invention, two or more corrugation panels are laterally coupled together to form a single continuous plurality panel. In an embodiment, 15 said coupling comprises one or more of adhesives, diffusion bonding, brazing, soldering or resistance/electron/laser welding, or friction stir welding. FIG. 15(A) depicts a schematic representation of friction stir welding. FIG. 15(B) depicts a schematic of two or more truss based structures 20 1503 coupled together to form a plurality panel 1509 containing, in illustration shown, five sets of the corrugation panels with the corresponding facesheets 1504, truss unit portions 1505, nodes 1506, vertical side members 1510, legs or ligaments 1511, and weld lines 1512, etc. The extruded corrugation panels can take on a variety of shapes, dependent only upon the desired topology of the final sandwich structure or any desired/required structure. FIG. 15(B) depicts the corrugation panels of truss based structures 1503 with prismatic core shapes. It is envisioned, however, that tetrahedral, 25 Kagome, cone, frustum, or other truss structures may be manufactured via this method. FIG. 15(B) depicts vertical side members 1510 that are substantially planar. It is envisioned, however that the vertical side members 10 can take on any variety of widths and shapes such as substantially 30 C-shaped or L-shaped. The truss in FIG. 15(B) units 1505 comprise of a plurality of legs or ligaments 1511. FIG. 15(B) depicts the legs or ligaments 1511 as straight. It is envisioned however, that the legs may have a variety of shapes such as straight or curved and may have a variety of cross-sections. In 35 an embodiment the monolithic samples may comprise at least one select material as desired or required. In an embodiment, the select material may comprise, for example, but not limited thereto, ceramic, polymer, metal, metal alloy, and/or any combination of composites thereof (or any material(s) as 40 desired or required. The area that the facesheet or faceplate and truss units intersect form an interface region. In an embodiment, the interface region has the same metallurgical and microstructural properties. In an embodiment, the truss units have nodes wherein the nodes have the same metallurgical and 45 microstructural properties as the truss unit. In an embodiment, the extruding or machining or both the extruding and machining create the truss units of varying relative density. In an embodiment, the nodes have curved or smooth triple point interfaces with the facesheets.

FIG. 16(A) provides a photographic depiction of a plurality panel 1509 (having five truss based structures 1503 in this instance) comprising 6061-T6 aluminum corrugation panels, coupled by friction stir welding. The corrugation panels of the truss based structures 1503 were extruded from 6061 aluminum alloy and contain weld lines 1512, with facesheets 1504 enclosing truss units 1505, forming nodes 1506 where truss legs or ligaments 1511 interfaces with a facesheets 1504 at nodes 1506. FIG. 16(B) provides a magnified photographic depiction of a portion of the plurality panel 1509 depicted in FIG. 16(A) centered on a weld line 1512. The plurality panel in depicted in FIG. 16(B) contains weld lines 1512, with facesheets 1504 enclosing truss units 1505, forming nodes

## 15

1506 where truss legs or ligaments 1511 interfaces with a facesheets 1504 at nodes 1506. FIG. 16(B) shows that the plurality panel has the following dimensions: a vertical side member thickness of 9.5 mm, a core height of 19.05, and 5.4 mm thick facesheets. It should be appreciated that the dimension, contours, thicknesses, and sizes may vary as desired or required for particular structure, application, or process.

Next, although not shown, in an exemplary and non-limiting embodiment of an aspect of the present invention, these manufacturing techniques may be used to form multi-layered plurality panels, by vertically coupling said plurality panels. Said vertical coupling can comprise claiming, adhesives, diffusion bonding, brazing, soldering or resistance/electron/laser welding, or friction stir welding. Again, the following is a description for the manufacture of a double-layer pyramidal/triangular corrugation plurality panel, however, it is envisioned that tetrahedral, Kagome, cone, frustum, or other lattice-based truss structures of any number of layers may be manufactured via this method. The combination of these two steps produces a multi-layered (in the at least substantially vertical direction) corrugated extrusion plurality panel, with facesheets enclosing truss units, forming nodes where truss legs or ligaments interface with a facesheet at nodes, and containing weld lines. It is noted that the alignment of nodes 6 between adjacent layers is not a prerequisite. As with this embodiment or any embodiments discussed herein, each individual layer may be aligned or offset any amount from adjacent layers, yielding the desired properties for the structure as a whole and the layers individually. Similarly, the truss units may have any number of legs or ligaments according to the fabrication approach. The truss units 1505 comprise of a plurality of legs or ligaments 1511. The legs may have a variety of shapes such as straight or curved and may have a variety of cross-sections. The plurality of truss units 1505 form an array of truss units. While the y-direction path and the x-direction path are shown as substantially straight, it should be appreciated that the paths may be curved or shaped as desired or required. Moreover, while the various extrusion paths (x, y, and z) as illustrated appear to be substantially orthogonal or perpendicular respectively with one another, it should be appreciated that any respective angles may be implemented as desired or required for the desired or required fabrication process or resultant truss and/or panel structure. For instance, the array of truss units and panels (or any related components of the resultant structure) may be fabricated so that the truss units and panels (or any related components) may be contoured or shaped as desired or required. In an embodiment, the monolithic sample may comprise at least one select material as desire or required. In an embodiment, the select material may comprise, for example but not limited thereto, aluminum, ceramic, polymer, metal, metal alloy, and/or any combination of composites thereof (or any material(s) as desired or required. It should be appreciated that the monolithic sample may be extruded along a plurality of paths, such as two or more as desired or required. The area that the faceplate/facesheet and truss units intersect form an interface region. In an embodiment, the interface region has the same metallurgical and microstructural properties. In an embodiment, the truss units have nodes wherein the nodes have the same metallurgical and microstructural properties as the truss unit. In an embodiment, the extruding or machining or both the extruding and machining create the truss units of varying relative density.

Aspects of various embodiments of the present invention provide, but are not limited to, a novel method and system to manufacture corrugation truss based plurality panels or any desired/required structures that provides enhanced truss-

## 16

facesheet interface strength by avoiding poor joint design or bonding procedures, which can cause the catastrophic failure of sandwich panels. Although numerous factors determine the robustness of joined nodes (joint composition, microstructure, degree of porosity, geometric constraints, etc.) this new method results in sandwich structures with highly robust nodes that have the equivalent metallurgical, for instance strength, ductility, chemical composition, microstructural characteristics, etc. of the parent material. Aspects of the present invention methods can be used for, but are not limited to, any solid, metal, or metal alloy, including, but not limited to, steels, aluminum, copper, magnesium, nickel, titanium alloy, etc. and is highly suited for alloys which possess limited ambient temperature ductility.

15 This approach can be extended to other material classes. For example, various approaches have been developed for producing polymeric structures with prismatic cores that can then be fabricated via the means described heretofore, including truss based sandwich structures. Ceramic materials with 20 prismatic cores can also be fabricated using “green state” extrusion forming and sintering, in which the material can be laterally machined prior to or after a sintering operation. Edge-defined film fed growth also provides a means for fabricating prismatic structures of the type envisioned here from 25 many types of materials, including ceramics (sapphire for example) and semiconductors (such as silicon).

It should be appreciated that prior to or after any extrusions 30 the sample, billet, panel, or structure may be fabricated or manipulated by machining (e.g., machined via electro discharge machining), cutting or any other suitable operation as discussed in U.S. patent application Ser. No. 12/447,166, filed Apr. 24, 2009, entitled “Manufacture of Lattice Truss Structures from Monolithic Materials” and it’s corresponding PCT International Application No. PCT/US/2007/022733, filed Oct. 26, 2007; of which the disclosures are hereby incorporated by reference herein in their entirety.

## EXAMPLES

## Example and Experimental Results Set No. 1

Practice of the invention will be still more fully understood from the following examples and experimental results, which are presented herein for illustration only and should not be construed as limiting the invention in any way.

An aspect of an embodiment of this invention may comprise an extrusion and electro discharge machining (EDM) method has been developed to fabricate a pyramidal lattice core sandwich structure. The approach is readily extendable 50 to tetrahedral and to multilayer versions of these lattices. In this approach, a 6061 aluminum alloy corrugated core sandwich panel is first extruded, creating an integral core and facesheets, fashioned from a single sample of material. The corrugated core (or any core shape as desired or required) is 55 then penetrated by an alternating pattern of triangular shaped EDM electrodes normal to the extrusion direction to form the pyramidal lattice. The process results in a sandwich panel in which the core-facesheet nodes possess the parent materials’ metallurgical and mechanical properties. The out-of-plane compression and in-plane shear mechanical properties of the structure have been measured and found to be very well predicted by analytical estimates.

Referring to FIG. 5, a sample 41, such as an extrusion billet for example, comprising 6061 aluminum alloy, was extruded 60 with a regular prismatic structure using extrusion press 43 (as schematically shown by the dotted lines) by a heat source 42. In this example the heat is applied at 482° C. and the press 43

(having flow channels 45) has a dimension of 17.8 cm diameter, 300 ton direct extrusion press at 482° C., resulting in a corrugated core sandwich panel structure 44, such as a long extrusion stick.

Referring to FIG. 6(A), after this extrusion step (as shown in FIG. 5), the resulting corrugated core sandwich panel structure 44 had a web thickness of 3.2 mm as designated by arrow WT, a core height of 19.1 mm as designated by the arrow CH, and a facesheet thickness of 5.2 mm as designated as FT and a web inclination angle of 60° as designated by arrow WI. The relative density of the corrugated core was 25%. The extruded panels were solutionized, water-quenched and heat-treated to a T6 condition. An alternating pattern of triangular shaped EDM electrodes (not shown) were then inserted normal to the extrusion direction as illustrated in FIG. 6(A) as the patterns to be removed 51 to form the pyramidal lattice sandwich panel, as shown FIG. 6(B). The triangular plates are shown as cutouts 52 that are perpendicular to the extrusion. The process resulted in a sandwich panel in which the core-facesheet nodes 13 had identical microstructure, composition and mechanical properties to those of the trusses 14 and facesheets 11.

It should be appreciated that any dimensions or angles shown herein are exemplary and illustrative only and should not be construed as limiting the invention in any way. The sizes, materials, flexibility, rigidness, shapes, contours, angles or dimensions discussed or shown may be altered or adjusted as required or desired.

FIG. 7 shows a photographic depiction of one of the pyramidal lattice sandwich structures. It is 4 unit cells wide by 4 unit cells long as shown by the respective truss-units 12, and was used for compression measurements. The shear response was measured using samples (not shown) that were 4 unit cells wide and 10 unit cells long.

#### Test Results

The relative density can be derived for the pyramidal structure depends upon the truss cross sectional area,  $t^2$ , its inclination angle,  $\omega$ , and length,  $l$ . The ratio of the metal volume in a unit cell to that of the unit cell then gives the relative density:

$$\rho = \frac{2t^2}{l^2 \sin \omega \cos^2 \omega} \cdot \frac{l^2 \cos^2 \omega}{(l \cos \omega + \sqrt{2} t)^2} \quad (1)$$

For the samples manufactured here,  $t=3.2$  mm,  $l=24.6$  mm and  $\omega=50.77^\circ$  resulting in a predicted relative density of 6.5%. The experimentally measured relative density was  $6.2 \pm 0.01\%$ .

The lattice truss structures were tested at ambient temperature in compression and shear at a nominal strain rate of  $10^{-2}$   $s^{-1}$  in accordance with ASTM C365 and C273 using a compression shear plate configuration. A laser extensometer measured the compressive strain by monitoring the displacements of the unconstrained facesheets (with a displacement precision of  $\pm 0.001$  mm. The shear strain was obtained by monitoring the displacements of the shear plates with a measurement precision of  $\pm 0.010$  mm.

Referring to FIG. 8, the through thickness compressive stress-strain response pertaining to the pyramidal lattice sandwich structure substantially shown in FIG. 7 is graphically shown in FIG. 8(A). FIGS. 8(B)-(G) show photographic depictions of the lattice deformation at strain levels ( $\epsilon$ ) of 0, 5, 10, 15, 20 and 25%, respectively. Following an initial linear response, a peak was observed in the compressive stress that coincided with initiation of the buckling of the lattice truss

members and the formation of a plastic hinge near the center of the truss members. Continued loading resulted in core softening up to an engineering strain of  $\sim 0.25$  at which point the load carrying capacity increased rapidly as the deformed trusses made contact with the facesheets. During the core-softening phase, small fractures were observed to form on the tensile stressed side of the trusses. These were first seen at strains of between 0.10 and 0.12. No failures at the truss-facesheet nodes were observed during any of the tests.

Referring to FIG. 9(A), the in-plane shear stress-strain response pertaining to the pyramidal lattice sandwich structure substantially shown in FIG. 7 is graphically shown in FIG. 9(A). FIGS. 9(B)-(D) show photographic depictions of the lattice deformation at strain levels ( $\gamma$ ) of 0, 6 and 12%, respectively. In this test orientation, each unit cell had two truss members loaded in compression and two in tension. The sample exhibited characteristics typical of lattice truss based sandwich cores including: elastic behavior during initial loading and increasing load support capability until the peak strength was reached. Continued loading continued at a constant stress up to a strain of  $\sim 0.13$ , at which point the sample failed by fracture of the tensile loaded lattice members near their midpoint. Some plastic buckling was observed on truss members at the ends of the sandwich panel. It is a manifestation of the compressive loading component of the ASTM 273 test method. No evidence of node failure was observed during any of the shear experiments.

Tensile coupons of the aluminum 6061 alloy were used to determine the mechanical properties of the parent aluminum alloy. Tensile tests were performed according to ASTM E8 at a strain rate of  $10^{-3}$   $s^{-1}$ . The average Young's modulus,  $E_s$ , and 0.2% offset yield strength,  $\sigma_{ys}$ , were 69 GPa and 268 MPa, respectively. The tangent modulus,  $E_t$ , at the inelastic bifurcation stress was 282 MPa.

The peak strength of a lattice truss core is determined by the mechanism of strut failure which, in turn, depends on the cell geometry, strut material properties and the mode of failure loading. Table 1 summarizes the micromechanical predictions for the pyramidal lattice. The micromechanical predictions for the compressive and shear peak strength are shown in FIGS. 8(A) and 9(A) for truss members that fail by plastic yielding or inelastic buckling. There is excellent agreement between the analytical model predictions of the peak strengths and the observed modes of deformation.

The compression and shear stiffnesses were measured from periodic unload/reload measurements. FIG. 10(A) graphically shows the non-dimensional compressive stiffness,  $\Pi = E_c / (E_s \bar{\rho})$ , versus compressive strain (here  $E_c$  and  $E_s$  are the Young's moduli of the core and the solid parent alloy respectively, and  $\bar{\rho}$  is, again, the relative density). The predicted non-dimensional compressive stiffness is 0.36. The experimental data fall slightly above 0.36 just prior to attainment of the peak strength and then decrease during the inelastic buckling phase of deformation. FIG. 10(B) graphically shows the non-dimensional shear stiffness,  $\Gamma = G_c / (E_s \bar{\rho})$ , versus shear strain (here  $G_c$  is the shear stiffness of the core). The predicted non-dimensional shear stiffness of 0.12 and the experimental data are in excellent agreement up until failure of the panel.

Table 1 provides the analytical expressions for the compression and shear stiffness and strength of a pyramidal lattice truss core sandwich structure.

TABLE 1

| Mechanical Property:                      | Analytical Expression:                                                            |
|-------------------------------------------|-----------------------------------------------------------------------------------|
| Compressive stiffness                     | $E_c = \bar{\rho} E_s \cdot \sin^4 \omega$                                        |
| Compressive strength (plastic yielding)   | $\sigma_{pk} = \bar{\rho} \sigma_{ys} \cdot \sin^2 \omega$                        |
| Compressive strength (inelastic buckling) | $\sigma_{pk} = \bar{\rho} \sigma_{cr} \cdot \sin^2 \omega$                        |
| Shear stiffness                           | $G_c = \bar{\rho} \cdot \frac{1}{8} E_s \cdot \sin^2 2\omega$                     |
| Shear strength (plastic yielding)         | $\tau_{pk} = \bar{\rho} \cdot \frac{1}{2\sqrt{2}} \sigma_{ys} \cdot \sin 2\omega$ |
| Shear strength (inelastic buckling)       | $\tau_{pk} = \bar{\rho} \cdot \frac{1}{2\sqrt{2}} \sigma_{cr} \sin 2\omega$       |

A new method for fabricating a lattice truss core sandwich panel structure has been developed using a combination of extrusion and electro discharge machining. The approach has been illustrated by the fabrication and mechanical property evaluation of sandwich panels made from a 6061 aluminum alloy; however, the method is applicable to any alloy system that can be easily extruded. For materials that can not be extruded, the electro discharge machining method could be performed in two directions (instead of one as described here) on a monolithic plate resulting in a similar lattice structure. This alternative method, therefore, is extendable to most conductive material systems or other material systems as desired or required.

The measured peak compressive and shear strengths were found to be in excellent agreement with the micromechanical model predictions for the operative truss member failure mechanisms: inelastic buckling for compression and plastic yielding (followed by tensile fracture) for shear. The non-dimensional compression and shear moduli coefficients were found to be in excellent agreement with the analytical predictions.

Conventional sandwich panel structures suffer from node failure during static and dynamic testing. These failures are initiated at defects or in weak or embrittled regions that result from core-faceplate bonding (facesheet bonding) processes. Whereas, the present invention fabrication method described above, results in sandwich panels in which the core-facesheet nodes have identical material properties to those of the trusses and facesheets. Joining methods such as brazing or welding have been eliminated with this process. No evidence of nodal failure was observed during compression or shear loading of the samples fabricated by the method described here.

The method of sandwich panel manufacture described here has been used to fabricate sandwich panels that eliminate the incidence of nodal failures. The panels' mechanical properties are found to be governed only by the geometry of the sandwich panel, the alloy mechanical properties, and the mode of loading. These properties are well predicted by recent micromechanical models.

#### Example and Experimental Results Set No. 2

An aspect of an embodiment of this invention may comprise an extrusion developed to fabricate a pyramidal corrugation truss based corrugation panels, laterally coupled by a process comprising friction stir welding to form corrugation plurality panels. The approach is readily extendable to tetrahedral and to multilayer versions of these trusses. In this

approach, multiple 6061 aluminum alloy corrugated core sandwich panels is first extruded, creating an integral cores and facesheets, fashioned from a single samples of material. The corrugated cores (or any core shape as desired or required) are then laterally coupled by friction stir welding to form a continuous plurality panel. The process results in a sandwich panel in which the core-facesheet nodes posses the parent materials' metallurgical and mechanical properties. The out-of-plane compression and in-plane shear mechanical properties of the structure have been measured and found to be very well predicted by analytical estimates.

Referring to FIG. 14(A), a sample 1514, such as an extrusion billet 14 for example, comprising 6061 aluminum alloy, was extruded with a regular prismatic structure using extrusion press 1516 (as schematically shown by the dotted lines) by a heat source 1515. In this example the heat is applied at 482° C. and the press 1516 (having flow channels 1518) has a dimension of 17.8 cm diameter, 300 ton direct extrusion press at 482° C., resulting in a corrugated core sandwich panel structure 1517, such as a long extrusion stick. It should be appreciated that the temperature, dimension and force may vary as desired or required for particular structure or process.

Referring to FIG. 14(B), after this extrusion step (as shown in FIG. 14(A)), the resulting corrugated core sandwich panel structure 1503 had a web thickness of 0.125 in, a core height of 0.75 in, 0.216 in thick facesheets and a web inclination angle of 60 degrees. The relative density of the corrugated core was 29%. The extruded panels were solutionized, water-quenched and heat-treated to a T6 condition. Plurality panels 30 were formed by laterally coupling these corrugation panels by friction stir welding. Referring to FIG. 16(A) five corrugation panels welded by friction stir welding to create corrugation plurality panels containing 0.37 mm thick vertical side members. Plurality panels as depicted in FIG. 16(A) were used in mine blast testing experiments.

It should be appreciated that any dimensions or angles shown herein are exemplary and illustrative only and should not be construed as limiting the invention in any way. The sizes, materials, flexibility, rigidness, shapes, contours, angles or dimensions discussed or shown may be altered or adjusted as required or desired.

#### Test Results—Mine Blast Simulation

A "Black Widow" blast testing rig (the "Rig") was used to measure the performance of the corrugation plurality panels 45 1509 described above and as shown in FIG. 16(A). FIG. 18(A) depicts a diagram of the Rig. The perimeter of the corrugation plurality panel 1509 was clamped to 0.75 in thick steel back support plate that lay underneath the corrugation plurality panel and a clamping plate that lay on top of the plurality panel. FIG. 18(B) provides a photograph of the Rig 50 with the "wet sand" charge (the "charge") at a standoff distance of 19 cm. The charge is made of 375 grams of C-4 explosive enclosed in a spherical shell having a diameter of 80 mm. In addition to the C-4 explosive, the remaining volume 55 of the shell was filled with 2.466 kg of 200 μm diameter glass spheres to simulate sand and 0.617 kg of water. FIGS. 18(C)-(H) provide a schematic depicting the process for constructing the charge. The tests were performed at four standoff distances: 15, 19, 22, and 25 cm. Corrugation plurality panel 60 performance at each standoff distance was compared against equivalent mass monolithic 6061-Al plates ("monolithic plates") that were 17 mm thick. FIG. 17(A) graphs hardness of the corrugation plurality panels in MPa as a function of distance from the weld. A weld line 1512, for example, is highlighted in FIG. 16(A). FIG. 17(A) shows that the hardness drops off sharply within 1 cm of the weld line from approximately 390 MPa at approximately 2 cm away from the

weld line all the way down to approximately 270 MPa at the weldline. FIG. 17(B) graphs the true stress in MPa as a function of true strain for both the parental material (i.e. 6061 aluminum alloy) and the friction stir welded ("FSW") 6061 aluminum alloy. The true stress for both the friction stir welded material and the parental material begins level off at an approximately true strain of approximately 0.01.

FIG. 19(A) provides a graph of back facesheet deflection after the charge detonation for both the corrugation plurality panels and the monolithic plates at each of the respective standoff distances. FIG. 19(B) provides the same information in a tabular form. The corrugated plurality panel "failed" at the 15 cm standoff as the back facesheet was displaced by 55 mm. The mass equivalent monolithic plate by contrast did not fail and the back facesheet deflection was 47 mm. However, for each of the other charge standoff distances, the corrugated plurality panel 1509 had smaller back facesheet deflections than did the mass equivalent monolithic plates at the corresponding charge standoff distances as shown in FIGS. 19(A) and (B).

FIG. 20(A) shows post blast photographs of the corrugation plurality panels 1509 at each of the charge standoff distances (15, 19, 22, and 25 cm) and FIG. 20(B) shows post blast photographs of the mass equivalent monolithic plates at each of the charge standoff distances (15, 19, 22, and 25 cm).

FIGS. 21(A) and (B) show post blast photographs of a corrugation plurality panel 1509 after subjection to charge detonation at 25 cm standoff. FIG. 21(A) shows some tearing along the region of the corrugation plurality panel 1509 that was clamped to the clamping plate and the back support plate ("clamped region") in the direction parallel to corrugations. However, there was no crack propagation along the weld. FIG. 21(B) shows photographs of the cross section of the corrugation plurality panel 1509 of FIG. 21(A), which displays the post blast displacement.

FIGS. 22(A) and (B) show post blast photographs of a corrugation plurality panel 1509 at a standoff distance of 22 cm. FIG. 22(A) shows tearing along the edge of the weld in the direction parallel to corrugations. FIG. 22(B) shows cross sections of the corrugation plurality panel 1509 of FIG. 22(A), which displays the post blast displacement.

FIGS. 23(A) and (B) show post blast photographs of a corrugation plurality panel 1509 at a standoff distance of 19 cm. FIG. 23(A) shows tearing along edge of weld in direction parallel to corrugations. FIG. 23(B) shows cross sections of the corrugation plurality panel 1509 of FIG. 23(A) having an edge with partial tearing that displays the post blast displacement.

FIGS. 24(A) and (B) show post blast photographs of a corrugation plurality panel 1509 at a standoff distance of 15 cm. FIG. 24(A) shows catastrophic failure in the center of corrugation plurality panel 1509 of FIG. 24(A) having an edge with tearing in the direction perpendicular to the corrugations. FIG. 24(B) shows cross sections of the corrugation plurality panel 1509 that displays the post blast displacement.

The table of FIG. 25 summarizes the failure modes of the corrugated plurality panels at each of the charge standoffs described above.

#### REFERENCES CITED

The following patents, applications and publications as listed below and throughout this document are hereby incorporated by reference in their entirety herein. The devices, systems, articles of manufacture and methods of various embodiments of the present invention disclosed herein may

utilize aspects disclosed in the following patents and applications and are hereby incorporated by reference in their entirety:

PCT International Application No. PCT/US02/17942, 5 entitled "Multifunctional Periodic Cellular Solids And The Method of Making Thereof," filed Jun. 6, 2002, and corresponding U.S. application Ser. No. 10/479,833, entitled "Multifunctional Periodic Cellular Solids And The Method of Making Thereof," filed on Dec. 5, 2003.

10 PCT International Application No. PCT/US03/16844, entitled "Method for Manufacture of Periodic Cellular Structure and Resulting Periodic Cellular Structure," filed May 29, 2003, and corresponding U.S. application Ser. No. 10/515,572, entitled "Multifunctional Periodic Cellular Solids And The Method of Making Thereof," filed Nov. 23, 2004.

15 PCT International Application No. PCT/US04/04608, entitled "Methods for Manufacture of Multilayered Multifunctional Truss Structures and Related Structures Therefrom," filed Feb. 17, 2004, and corresponding U.S. application Ser. No. 10/545,042, entitled "Methods for Manufacture of Multilayered Multifunctional Truss Structures and Related Structures Therefrom," filed Aug. 11, 2005.

20 PCT International Application No. PCT/US01/22266, entitled "Method and Apparatus For Heat Exchange Using Hollow Foams and Interconnected Networks and Method of Making the Same," filed Jul. 16, 2001, and corresponding U.S. application Ser. No. 10/333,004, entitled "Heat Exchange Foam," filed Jan. 14, 2003.

25 PCT International Application No. PCT/US01/25158 entitled "Multifunctional Battery and Method of Making the Same", filed Aug. 10, 2001, and corresponding U.S. application Ser. Nos. 10/110,368, entitled "Multifunctional Battery and Method of Making the Same", filed Jul. 22, 2002, and Ser. No. 11/788,958, entitled "Multifunctional Battery and Method of Making the Same", filed Apr. 23, 2007.

30 PCT International Application No. PCT/US03/27606, entitled "Method for Manufacture of Truss Core Sandwich Structures and Related Structures Thereof," filed Sep. 3, 2003, and corresponding U.S. application Ser. No. 10/526,296, entitled "Method for Manufacture of Truss Core Sandwich Structures and Related Structures Thereof," filed Mar. 1, 2005.

35 40 PCT International Application No. PCT/US01/17363, entitled "Multifunctional Periodic Cellular Solids And The Method of Making Thereof," filed May 29, 2001, and corresponding U.S. application Ser. No. 10/296,728, entitled "Multifunctional Periodic Cellular Solids And The Method of Making Thereof," filed Nov. 25, 2002.

45 PCT International Application No. PCT/US2007/012268, entitled "Method and Apparatus for Jet Blast Deflection", filed May 23, 2007 and corresponding U.S. application Ser. No. 12/301,916, entitled "Method and Apparatus for Jet Blast Deflection," filed Nov. 21, 2008.

50 PCT International Application No. PCT/US03/23043 and corresponding U.S. application Ser. No. 10/522,068, filed Jan. 21, 2005, entitled "Method for Manufacture of Cellular Materials and Structures for Blast and Impact Mitigation and Resulting Structure."

55 PCT International Application No. PCT/US2003/027605 and corresponding U.S. application Ser. No. 10/526,416, filed Mar. 2, 2005, entitled "Blast and Ballistic Protection Systems and Methods of Making Same."

60 65 ASTM C273 Standard Test Method for Shear Properties of Sandwich Core Materials. West Conshohocken, Pa., USA: ASTM International, 2006.

ASTM. C365 Standard Test Method for Flatwise Compressive Properties of Sandwich Cores. West Conshohocken, Pa., USA: ASTM International, 2006.

ASTM. E8 Standard Test Methods for Tension Testing of Metallic Materials. West Conshohocken, Pa., USA: ASTM International, 2006.

Bitzer, T. 1997 Honeycomb technology. London: Chapman & Hall.

Chiras, S., Mumm, D. R., Evans, A. G., Wicks, N., Hutchinson, J. W., Dharmasena, K. P., Wadley, H. N. G. and Fichter, S., 2002. The structural performance of near-optimized truss core panels. *International Journal Solids and Structures*, 39 (15) 4093-4115.

Cote, F., Deshpande, V. S. and Fleck, N. A., Shear fatigue strength of a prismatic diamond sandwich core. *Scripta Materialia* 2007; 56:585-588.

Cote, F., Fleck, N. A. and Deshpande, V. S., Fatigue performance of sandwich beams with a pyramidal core. *International Journal of Fatigue* 2007; 29:1402-1412.

Deshpande, V. S., Fleck, N. A. and Ashby, M. F., 2001. Effective properties of the octet-truss lattice material. *Journal of the Mechanics and Physics of Solids*, 49 (8), 1747-1769.

Deshpande, V. S. and Fleck, N. A., 2001. Collapse of truss core sandwich beams in 3-point bending. *International Journal of Solids and Structures*, 38 (36-37), 6275-6305.

Evans, A. G., Hutchinson, J. W. and Ashby, M. F., Cellular metals. *Current Opinion in Solid State and Materials Science* 1998; 3:288-303.

Evans, A. G., Hutchinson, J. W., Fleck, N. A., Ashby, M. F. and Wadley, H. N. G., The topological design of multifunctional cellular metals. *Progress in Materials Science* 2001; 46:309-327.

Gibson, L. J. and Ashby M F. Cellular Solids, Structure and Properties. Cambridge: Cambridge University Press, 1997.

Kooistra, G. W., Aluminum alloy lattice truss structures. *Materials Science & Engineering*, M. S. Charlottesville: University of Virginia, 2006.

Kooistra, G. W., Queheillalt D. T. and Wadley H. N. G., Shear behavior of aluminum lattice truss sandwich panel structures. *Materials Science and Engineering A* 2007; In Press. Lim, J. H. and Kang, K. J., 2006. Mechanical behavior of sandwich panels with tetrahedral and Kagome truss cores fabricated from wires. *International Journal of Solids and Structures*, 43 (17), 5228-5246.

McShane, G. J., Radford, D. D., Deshpande V. S. and Fleck, N. A., 2006. The response of clamped sandwich plates with lattice cores subjected to shock loading. *European Journal of Mechanics—A/Solids*, 25 (2), 215-229.

Queheillalt, D. T. and Wadley, H. N. G., 2005. Pyramidal lattice truss structures with hollow trusses. *Materials Science and Engineering A*, 397 (1-2), 132-137.

Queheillalt, D. T. and Wadley, H. N. G., Titanium Alloy Lattice Truss Structures. *Materials and Design* 2007: Submitted March 2007.

Radford, D. D., Fleck N. A. and Deshpande, V. S., 2006. The response of clamped sandwich beams subjected to shock loading. *International Journal of Impact Engineering*, 32 (6), 968-987.

Rathbun, H. J., Wei, Z., He, M. Y., Zok, F. W., Evans, A. G., Sypeck, D. J. and Wadley, H. N. G., 2004. Measurement and Simulation of the Performance of a Lightweight Metallic Sandwich Structure with a Tetrahedral Truss Core. *Journal of Applied Mechanics*, 71 (3), 305-435.

Sugimura, Y., 2004. Mechanical response of single-layer tetrahedral trusses under shear loading. *Mechanics of Materials*, 36 (8), 715-721.

Sypeck, D. J. and Wadley, H. N. G., 2002. Cellular metal truss core sandwich structures. *Advanced Engineering Materials*, 4 (10), 759-764.

Wadley, H. N. G., Multifunctional periodic cellular metals. *Philosophical Transactions of the Royal Society A: Mathematical, Physical and Engineering Sciences* 2006; 364: 31-68.

Wadley, H. N. G., Fleck, N. A. and Evans, A. G., Fabrication and structural performance of periodic cellular metal sandwich structures. *Composites Science and Technology* 2003; 63:2331-2343.

Wallach, J. C. and Gibson, L. J., 2001. Mechanical behavior of a three-dimensional truss material. *International Journal of Solids and Structures*, 38 (40-41), 7181-7196.

Wang, J., Evans, A. G., Dharmasena, K. and Wadley, H. N. G., 2003. On the performance of truss panels with Kagome cores. *International Journal of Solids and Structures* 40 (25), 6981-6988.

Zhou, J., Shrotiriy, P. and Soboyejo, W. O., 2004. On the deformation of aluminum lattice block structures from struts to structure. *Mechanics of Materials*, 36 (8), 723-737.

Zok, F. W., Waltner, S. A., Wei, Z., Rathbun, H. J., McMeeking, R. M. and Evans, A. G., 2004. A protocol for characterizing the structural performance of metallic sandwich panels: application to pyramidal truss cores. *International Journal of Solids and Structures* 41 (22-23) 6249-6271. European Patent No. 858,069 entitled "Extrusion of Metals". European Patent No. EP0 904,914 B1 to Sugiura, et al., entitled "Method for Forming a Molding".

U.S. Pat. No. 3,364,707 to Foerster entitled "Extrusion Forming Member and Method".

U.S. Pat. No. 4,878,370 to Fuhrman, et al., entitled "Cold Extrusion Process for Internal Helical Gear Teeth".

U.S. Pat. No. 1,365,987 to Hadfield, et al., entitled "Manufacture of Gun Tubes and Like Tubular Bodies".

International Patent Application Publication No. WO 2005/059187 A3 to Ungurean entitled "Solid Shapes Extrusion".

International Patent Application Publication No. WO 2005/059187 A2 to Ungurean entitled "Solid Shapes Extrusion".

International Patent Application Publication No. WO 02/088412 A3 to Michaluk entitled "Tantalum and Niobium Billets and Methods of Producing the Same".

International Patent Application Publication No. WO 02/088412 A2 to Michaluk entitled "Tantalum and Niobium Billets and Methods of Producing the Same".

U.S. Patent Application Publication No. 827,960 to Graham, et al., entitled "Improvements Relating to the Manufacture of Hollow Turbine or Compressor Blades".

U.S. Pat. No. 2,970,368 to Home entitled "Hollow Turbine or Compressor Blades".

U.S. Pat. No. 2,972,806 to Hignett, et al., entitled "Production of Turbine or Compressor Blades".

U.S. Pat. No. 4,373,241 to Maloof entitled "Method of Making Propeller Blade".

U.S. Pat. No. 6,305,866 B1 to Aota et al., entitled "Structure Joined by Friction Stir Welding".

U.S. Pat. No. 3,014,269 to Graham, et al., "Manufacture of Hollow Turbine Blades"

International Patent Application Publication No. WO 2008/153613 A2 to Ungurean entitled "Solid Shapes Extrusion".

U.S. Pat. No. 4,280,393 to Giraud et al., entitled "Light Weight Armored Vehicle."

In summary, while the present invention has been described with respect to specific embodiments, many modifications, variations, alterations, substitutions, and equivalents will be apparent to those skilled in the art. The present

invention is not to be limited in scope by the specific embodiment described herein. Indeed, various modifications of the present invention, in addition to those described herein, will be apparent to those of skill in the art from the foregoing description and accompanying drawings. Accordingly, the invention is to be considered as limited only by the spirit and scope of the following claims, including all modifications and equivalents.

Still other embodiments will become readily apparent to those skilled in this art from reading the above-recited detailed description and drawings of certain exemplary embodiments. It should be understood that numerous variations, modifications, and additional embodiments are possible, and accordingly, all such variations, modifications, and embodiments are to be regarded as being within the spirit and scope of this application. For example, regardless of the content of any portion (e.g., title, field, background, summary, abstract, drawing figure, etc.) of this application, unless clearly specified to the contrary, there is no requirement for the inclusion in any claim herein or of any application claiming priority hereto of any particular described or illustrated activity or element, any particular sequence of such activities, or any particular interrelationship of such elements. Moreover, any activity can be repeated, any activity can be performed by multiple entities, and/or any element can be duplicated. Further, any activity or element can be excluded, the sequence of activities can vary, and/or the interrelationship of elements can vary. Unless clearly specified to the contrary, there is no requirement for any particular described or illustrated activity or element, any particular sequence or such activities, any particular size, speed, material, dimension or frequency, or any particularly interrelationship of such elements. Accordingly, the descriptions and drawings are to be regarded as illustrative in nature, and not as restrictive. Moreover, when any number or range is described herein, unless clearly stated otherwise, that number or range is approximate. When any range is described herein, unless clearly stated otherwise, that range includes all values therein and all subranges therein. Any information in any material (e.g., a United States/foreign patent, United States/foreign patent application, book, article, etc.) that has been incorporated by reference herein, is only incorporated by reference to the extent that no conflict exists between such information and the other statements and drawings set forth herein. In the event of such conflict, including a conflict that would render invalid any claim herein or seeking priority hereto, then any such conflicting information in such incorporated by reference material is specifically not incorporated by reference herein.

We claim:

1. A method of creating a monolithic corrugation panel truss-based structure, said method comprising:  
 extruding a monolithic sample to obtain an extruded monolithic structure;  
 selectively removing material from said extruded monolithic structure to yield a first monolithic corrugation panel comprising two facesheets and a plurality of legs between and connecting said facesheets;  
 extruding another said monolithic sample to obtain another extruded monolithic structure;  
 selectively removing material from said another extruded monolithic structure to yield a second monolithic corrugation panel comprising two facesheets and a plurality of legs between and connecting said facesheets; and

laterally coupling said first and second monolithic corrugation panels to each other to form a single continuous panel structure.

2. The method of claim 1, further comprising coupling a third extruded monolithic corrugation panel to said first and second monolithic corrugation panels to form a single continuous panel structure.
3. The method of claim 2, wherein said coupling comprises at least one of bonding or welding.
4. The method of claim 3, wherein the said welding comprises friction stir welding.
5. The method of claim 2, wherein at least one of said coupled corrugation panels has a vertical side member located at the coupling interface between said at least one of said coupled corrugation panels and another of said coupled corrugation panels.
6. The method of claim 5, wherein said vertical side member is substantially planar.
7. The method of claim 5, wherein said vertical side member is substantially C-shaped or L-shaped.
8. The method of claim 5, wherein said vertical side member is thickened with respect to at least one other component of said at least one corrugation panel.
9. The method of claim 1, wherein said extruding creates at least one truss unit portion of a corrugation panel.
10. The method of claim 9, wherein said at least one truss unit portion comprises at least one node, wherein said at least one node has a curved or smoothed triple point interface with other components of said corrugation panels.
11. The method of claim 10, wherein at least one of said corrugation panels comprises:  
 at least one facesheet, and  
 wherein said curved or smooth triple point interface of said at least one node interfaces with said at least one facesheet.
12. The method of claim 1, wherein at least one of said corrugation panels comprises at least one facesheet.
13. The method of claim 1, wherein a monolithic sample comprises ceramic, polymer, metal, alloy, and/or any combination of composites thereof.
14. The method of claim 13, wherein said metal comprises aluminum.
15. The method of claim 1, wherein said first and second monolithic corrugation panels are vertically coupled.
16. The method of claim 15, wherein said vertical coupling comprises at least one of: clamping, welding, or bonding.
17. The method of claim 1, wherein said monolithic corrugation panel truss-based structure is in communication with at least one of a tank to provide tank armor plating structure, or a land, air, space or water vehicle/craft to provide land, air, space or water vehicle/craft plating structure for mitigating damage caused by at least one of blast pressure or ballistic threats.
18. A panel structure comprising: a first monolithic corrugated panel and a second monolithic corrugated panel comprising two facesheets and a plurality of legs between and connecting said facesheets, wherein said first and second monolithic panels are laterally coupled in communication with one another to form a single continuous panel structure, and wherein said panel is manufactured using the method as set forth in claim 1.